

A. Patterson.

Making Hoes.

No 25,580.

Patented Sept. 27, 1859.

Fig. 1.



Fig. 4.



Fig. 2.



Fig. 5.



Fig. 3.



Witnesses:

Charles Darr

Ino P. Barcroft

Inventor:

A. Patterson

# UNITED STATES PATENT OFFICE.

ANDREW PATTERSON, OF BIRMINGHAM, PENNSYLVANIA.

## MANUFACTURE OF HOES.

Specification of Letters Patent No. 25,580, dated September 27, 1859.

*To all whom it may concern:*

Be it known that I, ANDREW PATTERSON, of Birmingham, Allegheny County, State of Pennsylvania, have invented a certain new and useful Improvement in the Manufacture of Hoes; and I hereby declare that the following is a full and exact description thereof, reference being had to the accompanying drawings, which form part of this specification, and to the letters of reference marked thereon.

The nature of my invention consists in forming the head or eye of a hoe and attaching it at the same time to a sheet metal blade by pouring molten metal to form the head or eye, on or around the blade previously placed in a properly constructed mold.

The better to enable others to make hoes in accordance with my improvement I will more fully describe it in view of the drawings of which—

Figure 1 is a perspective of the back of a finished hoe. Fig. 2 is a perspective of the front of a finished hoe. Fig. 3 is a perspective of a vertical section through the head and blade showing the manner in which they are united. Fig. 4 is a perspective of a blade prepared to receive the molten head or eye. Fig. 5 is a perspective section of the blade, the position of the head and the manner of its union with the blade, being indicated by the dotted lines.

The same letters refer to like parts in all the drawings.

35 *a* is the blade.

*b* is the head.

*c c c c* is a collar or flange on the blade and is formed by bending up a part of the blade so as to allow the metal which forms the head to flow on or around it and clasp the blade and securely join the head and blade together.

It is not important that the blade should be cut or stamped exactly as shown at *c c c*. 45 This part may be varied to suit circumstances. The shape shown is a convenient and efficient one, the chief condition being such an arrangement relative to the head that the metal to form the head may so flow on that part of the blade as to securely unite the head and blade together.

In making hoes according to my improvement I proceed as follows: Having determined the shape and configuration of hoe 50 I desire to produce I prepare a pattern of the entire or perfect hoe and having molded

an impression from it in sand or other suitable material I take a plate of sheet metal of the proper size and shape and place it in the impression in the place of the pattern 60 blade, with the part *c c c c* (or its equivalent in other styles of hoe) so placed with reference to the head that the metal which forms the head may so flow on it as to securely join the head and blade together. I then close the mold and pour into it a quantity of molten metal sufficient to fill the unoccupied portion of the mold and form the remainder of the hoe, the molten head becoming firmly 65 united to the blade.

In making hoes by my improvement sheet steel is a suitable material for the blade and common cast iron for the head, but I do not wish to be confined to them.

I am aware that hoes have been made 75 with a sheet steel blade and a cast malleable head welded on, such construction being claimed by Saml. Boyd in his patent of Jan. 13, 1857, as a new manufacture. The 80 patent of Henry Havell, Feb. 10, 1857, is for a certain form of steel blade welded to a cast malleable head. My invention differs from both these, 1st, in the materials of which the hoe is formed. My hoe head may be made of common cast iron without any preparation and is attached in the process of formation. In both the cases above referred to (Boyd and Havell patents) the head, although formed by casting, cannot 85 be attached to the blade as they direct (by welding) until after it has been decarbonized or rendered malleable and then it does not differ from a hoe head of the same shape which is made by forging. My improvement further differs from those of Boyd and Havell in the fact that it pertains to a different art. In those cases the finished 90 hoe is the handiwork of a blacksmith or worker in wrought metals, in mine it is the handiwork of a founder or molder, the work of a different artisan, the product of a different art. Certainly I have affected the manufacture of hoes—I think as certainly 95 improved it.

I am aware that it is not new to cast one metal or material on another. The process is old in a variety of arts. Cast and wrought iron, brass and iron, lead and silver, glass and metals, enamel and metals and other substances have been connected by this process in the production of various articles of manufacture and all or nearly all 100 105 110

such combinations have been or are now the subject of various patents as applied to the production of various articles which were never before so produced, the invention 5 consisting not in the discovery of the process but in improving this or that art or manufacture by connecting with it a process never before connected with it. My invention consists not in the discovery of casting 10 one metal on another but in improving the manufacture of hoes by substituting this old process which was never before used in that manufacture for other processes which were previously used in it.

I therefore desire to claim as my invention—

The improvement in the manufacture of hoes, herein substantially described, viz: forming the head or eye of a hoe and attaching it to the blade at the same time by 20 pouring the molten metal to form the head on or around the blade substantially as described and set forth.

A. PATTERSON.

Witnesses:

CHAS. B. BARR,  
JNO. P. BARCROFT.